

Nov. 5, 1940.

H. M. BLAETZ

2,220,671

MANUFACTURE OF ELECTROTYPE PRINTING PLATES

Filed Oct. 16, 1937



INVENTOR

WITNESS:

Robt. R. Kitchell.

Harry M. Blaetz  
BY

Augustus B. Stoughton  
ATTORNEY.

## UNITED STATES PATENT OFFICE

2,220,671

## MANUFACTURE OF ELECTROTYPE PRINTING PLATES

Harry M. Blaetz, Haddonfield, N. J., assignor to  
 The Curtis Publishing Company, Philadelphia,  
 Pa., a corporation of Pennsylvania

Application October 16, 1937, Serial No. 169,389

2 Claims. (Cl. 101—401.3)

The principal object of the present invention is to so condition the plates during the process of manufacture that relative level differentials may be impressed into the face of the plate in 5 all areas, either large or small, that may require such differentials for the proper reproduction of the various tone values during the printing operation.

Other objects of the invention will appear 10 from the following description at the end of which the invention will be claimed.

Generally stated the invention consists in heating a partially completed electrotype plate to a critical temperature and then quenching or 15 suddenly cooling it, thereby developing in the backing-up lead alloy extreme softness followed after a time interval by increased hardness and toughness in respect to its initial condition, and thereafter and during said time interval and 20 while the plate is in softened condition imparting level differentials not only at relatively large but also and in addition at relatively small areas of the plate surface by the application of pressure and a mat or matrix corresponding to both 25 small and large surface areas of the plate.

The invention also consists in the improvements hereinafter described and finally claimed.

Heretofore it has been customary to "back-up" 30 a flat electrotype shell (nickel faced copper, both electro-deposited) with lead alloy bonded by tin foil, and to carry the flat plate through most of the operations involved in completing the plate. When it is necessary to "McKee treat" a plate this operation is also performed on the flat plate. 35 This McKee treatment consists of hot-pressing the level differentials which constitute the various tone gradations into the face of the plate, using a built-up matrix on the face and a female matrix on the back, as, for example, according to McKee Patents U. S. Numbers 988,583 and 40 1,077,621. This results in solid printing areas being raised, and high-light areas being relatively depressed, with areas of intermediate tone values forced to correspondingly intermediate 45 levels. The level differentials between the solid areas and high-light areas usually amount to some two to five one-thousandths of an inch. The flat plate is curved, for mounting on the printing press plate cylinder, as one of the final 50 operations in the plate making sequence. The plate may be curved either hot or cold.

Standard equipment now available in the market permits casting or backing up a curved shell and carrying the curved plate through the entire sequence of operations. Each machine used

has the same press-plate cylinder arc so that the completed plate will fit the cylinder perfectly. The equipment also provides for the McKee treating step when needed. This treatment may be applied by means of a laminated or built-up 5 face matrix in a curved-bed machine equipped with toothed rollers and is completed in a curved-bed shaving machine.

The operation of these machines on plates which must be McKee treated often results in a 10 serious disadvantage. These machines include pressure rollers used alone or in connection with cutting means, and a plate passing through these machines may be rolled as many as twelve times. This repeated rolling under pressure compacts 15 the plate alloy making it harder and tougher and making the grain finer. While this is of ultimate benefit to the plate in making it more 20 resistant to wear during the printing operation still it works against the application of proper 25 McKee treatment to the plate. By the time the McKee treating step has been reached the plate alloy is so hard that it is feasible to apply level-differentials only to comparatively large areas of plate surface. The treatment of small areas, 30 a quarter of an inch to half an inch in diameter, often necessary for satisfactory printed results must be and is neglected. In an attempt to correct this disadvantage another step has sometimes heretofore been introduced into the operation sequence and it consists in the use of a 35 machine that softens the plate by heating it to about 425° F. which is not a critical temperature. This, however, is only a make-shift.

Heat treating to a critical temperature and 40 then quenching or suddenly cooling the partially completed plate before rolling and shaving and McKee treating produces an extreme softness of the plate which persists for some two or three 45 hours and is then followed by a rapid toughening and hardening. The heat treating consists in heating the plate at a temperature of 470° F. more or less for about fifteen minutes followed by rapid cooling as by quenching at a temperature of about 45° to 65° F.

While the plate is in the extremely soft condition the remaining operations in the sequence 50 can be quickly and easily carried out. I have discovered and my invention is based on the discovery that this is particularly true of the McKee treatment step because the softness of the alloy readily permits the production of smoothly graded level differentials in any areas of the plate either large or small as may be required by the nature of the subject. This results in a 55

plate having superior printing qualities as compared with any other curved plate method with which I am familiar. Pages printed from such plates are substantial reproductions of the original plate that is used in the production of the nickel faced copper electrotype shell.

The heat treating step to a critical temperature with rapid cooling, of itself, insures subsequent hardening and toughening of the plate alloy with desirable fine grain structure and the pressure rolling of the plate in operations following such heat treatment is not disadvantageous because the extreme softness of the alloy persists over a period of time ample for carrying out the operations of completing the plate including the McKee treatment so that the rolling aids and accelerates the later toughening of the alloy and helps to put the plate into condition for properly withstanding the wearing and hammering action of long press runs.

It may be remarked that the step of heat treating to the critical temperature with sudden cooling or quenching is advantageous in the customary flat plate sequence. In that case such heat treating precedes the shaving of the plate, and the McKee treatment is combined with the shaving operation by using a built-up matrix on the face of the plate. The equipment used is a standard flat bed shaving machine having a series of spring pressed rollers operating with the shaving knife. The principle is exactly the same as that of the curved bed shaver used on curved plates. This contrasts with the necessity for applying the McKee treatment in a heated platen hydraulic press as an entirely separate operation. The extreme softness of the alloy resulting from heating to the critical temperature and suddenly cooling or quenching makes it possible to combine the McKee treating and shaving operations. This softness also improves the later curving of the plate resulting in a substantially perfect fit for the press cylinder with no tendency to resist the retention of the curved form. In heat treating an electrotype printing plate it is exposed to a high temperature—about 470° F. more or less—for about fifteen minutes, followed by rapid cooling, as by quenching at a temperature of about 45° to 65° F. usually by immersion in a fluid or liquid. In practice the temperature may rise sufficiently to soften the plate, so that if curved it tends to flatten out, and if flat it tends to assume curved or warped form, again the shell takes up or absorbs ambient heat more rapidly than the alloy which is a poor conductor of heat so that the shell expands more rapidly than the alloy, causing defects and disadvantages.

According to my invention the first of these difficulties may be avoided by the use of a support for the plate during the heat treatment and the support may be flat or curved; and the second of these difficulties may be avoided by interposing between the face of the support and the shell of the plate heat insulating or non-conducting material, or by otherwise covering the shell of the plate with such material. In cases where the plate is quenched by immersion the material used for covering purposes should be unaffected by the fluid in which the plate is

immersed. The heat-insulating or non-conducting material serves to minimize the heat absorbed by the shell of the plate and in that way opposes over heating it, and the support opposes deformation of the plate itself.

In the accompanying drawing:

Figure 1 is a perspective view of apparatus useful in applying rolling pressure to the back of a curved partially completed electrotype plate.

Figure 2 is a similar view of apparatus adapted to apply pressure and to trim or shave the back of the plate, and

Figure 3 is an enlarged view illustrating the toothed surface of the roll 3 in Figure 1.

Referring to the drawing, I indicated a curved machine whose cylinder 2 conforms to the press cylinder. As shown in Figure 1 this machine is provided with rollers 3 having toothed surfaces and they apply pressure at the back of the curved plate b. As shown in Figure 2 the machine comprises a series of spring pressed rollers 4 which precede a cutting knife 5 and the rollers and knife exert pressure when trimming or shaving at the back of the plate. When such machinery is used in the practice of the invention the mat or matrix is applied to the face of the plate b and it is made to produce level differentials corresponding or in consonance with the requirements of the proof of form in respect to gradations of light and shade over its entire surface including both large and small areas. This is made possible according to my invention because of the extreme softness of the alloy backing produced by critical heat treatment at a temperature of about 470° F. followed by rapid cooling or quenching as described.

It will be obvious to those skilled in the art to which the invention relates that modifications may be made in details of procedure and in matters of mere form without departing from the spirit of the invention which is not limited to such matters or otherwise than the prior art and the appended claims may require.

I claim:

1. The improvement in the process of making electrotype printing plates which consists in heating a partially completed electrotype plate to a critical temperature of about 470° F. for about fifteen minutes and then rapidly cooling it as by quenching at a temperature of about 45° to 65° F. thereby developing in the backing up lead alloy softness followed after a time interval by increased hardness and toughness in respect to its initial condition, and thereafter and during said time interval and while the plate is in softened condition imparting to it level differentials not only at relatively large but also at relatively small areas of the plate surface by the application of pressure and a mat or matrix corresponding to both small and large surface areas of the subject.

2. The improvement in the process of making electrotype printing plates which consists in subjecting them to heating and quenching thereby softening their lead alloy and while the lead alloy is soft pressing level differentials into the printing face with a mat or matrix corresponding with the subject.

HARRY M. BLAETZ.